

- [54] THIXOTROPIC METAL-CONTAINING MONOMETHYLHYDRAZINE FUEL AND METHOD OF PREPARING THE SAME
- [75] Inventor: Barry D. Allan, Huntsville, Ala.
- [73] Assignee: The United States of America as represented by the Secretary of the Army, Washington, D.C.
- [22] Filed: Jan. 3, 1966
- [21] Appl. No.: 518,489
- [52] U.S. Cl..... 149/20, 149/19.7, 149/21, 149/22, 149/36, 149/118
- [51] Int. Cl..... C06b 19/04, C06c 1/02
- [58] Field of Search..... 149/36, 18, 20, 44, 19.7, 149/21, 22, 118

- [56] References Cited
- UNITED STATES PATENTS
- 3,164,505 1/1965 Hsieh et al..... 149/36
- FOREIGN PATENTS OR APPLICATIONS
- 978,105 12/1964 Great Britain..... 149/36

Primary Examiner—Leland A. Sebastian  
Attorney, Agent, or Firm—Edward J. Kelly; Herbert Berl; James T. Deaton

#### EXEMPLARY CLAIM

A composition consisting of gelled monomethylhydrazine containing dispersed therein up to 70 weight per cent finely divided metallic fuel particles and a cellulose or hydroxyalkyl-substituted cellulose gelling agent.

6 Claims, 3 Drawing Figures



FIG. 1

Barry D. Allan,

INVENTOR.

Harry M. Saragovitz

BY Edward J. Kelly

Herbert Bell

Joseph H. Beumer



FIG. 2

Barry D. Allan,  
INVENTOR.

BY Harry M. Sargovitz  
Edward J. Kelly  
Herbert Berl  
Joseph N. Brunner

PATENTED DEC 31 1974

3,857,743

SHEET 3 OF 3



FIG. 3

Barry D. Allan,  
INVENTOR.

BY Harry M. Saragovitz  
Edward J. Kelly  
Herbert Beck  
Joseph H. Beumer

THIXOTROPIC METAL-CONTAINING  
MONOMETHYLHYDRAZINE FUEL AND METHOD  
OF PREPARING THE SAME

The invention described herein may be manufactured and used by or for the Government for governmental purposes without the payment of any royalty thereon.

This invention relates to rocket fuels and more particularly to gelled monomethylhydrazine containing metallic particles.

Monomethylhydrazine, commonly referred to as MMH, is useful as a liquid fuel for rocket motors. This material exhibits favorable combustion properties when reacted with an oxidizer such as nitric acid, a specific impulse,  $I_s$ , of 278 seconds (1,000 → 14 psia) being obtained. For applications where fuel-tank volume is limited, it is desired to increase the density of MMH while maintaining a high specific impulse. The effectiveness of the fuel in this regard is expressed in terms of specific impulse-density,  $\rho I_s$ , the product of density and specific impulse values. The specific impulse-density value for MMH — nitric acid is 355.8.

One means of increasing the specific impulse-density of MMH fuel is to provide finely divided particles of a metal such as aluminum in the MMH, this measure having been employed previously for solid propellants. Such an approach has not been practical for liquids such as MMH, however, owing to the difficulty of maintaining the particles in suspension. The fuel is normally stored in a tank on board the rocket for an extended period prior to firing, and the metal particles settle to the bottom of the liquid. The resulting inhomogeneity could not be tolerated in operation of the rocket motor. Stability of the metal-containing fuel is also adversely effected by vibration and acceleration forces encountered in flight of the rocket.

In order to maintain the metal particles in suspension and yet allow pumping of the fuel as a liquid the metal-containing MMH should be provided in the form of a thixotropic gel, which behaves as a stable solid until disturbed, but flows as a liquid when force is applied.

Provision of metal-containing MMH in the form of a thixotropic gel would also reduce the hazards associated with MMH. This material is highly toxic, and when handled in liquid form, extreme precautions must be taken to avoid leakage or escape of fumes. Furthermore, MMH reacts hypergolically with many common materials so that a leak could cause a disastrous fire. The reduced mobility of a gel as compared to liquid MMH would avoid these dangers.

It is therefore an object of this invention to provide a stable suspension of metallic fuel particles in MMH.

Another object is to provide a method of converting metal-containing MMH to a thixotropic gel.

Still another object is to provide a MMH rocket fuel having increased specific impulse-density.

Other objects and advantages will be apparent from the following detailed description.

In accordance with the present invention a thixotropic MMH gel containing metallic fuel particles is prepared by dispersing the fuel particles and a cellulose or hydroxyalkyl-substituted cellulose gelling agent in the MMH. The gelled, metal-containing MMH exhibits substantially increased specific impulse-density values, and the metal particles remain in suspension indefinitely. The gel can be pumped and fed into a rocket motor combustion chamber as a liquid by application

of moderate stress. The semi-solid character of this fuel minimizes the toxicity and fire hazards associated with handling and storage of liquid MMH.

Any cellulose or hydroxyalkyl-substituted gelling agent may be employed, and the following commercially available gelling agents, listed by their chemical composition and trade mark designation, are preferred: hydroxyl methyl cellulose containing 27.5 to 3.15 weight percent methoxyl groups, Methocel; hydroxypropyl methyl cellulose containing 28 to 30 weight percent methoxyl groups and 7 to 12 weight percent propoxyl groups, Methocel HG-60; hydroxypropyl methyl cellulose containing 19 to 24 weight percent methoxyl groups and 4 to 12 weight percent propoxyl groups, Methocel HG-90; dihydroxyethyl cellulose, Cellosize; and hydroxypropyl cellulose containing about 4.6 propoxyl groups per glucose unit, Klucel.

The gelling agent is provided in an amount sufficient to impart thixotropic character to the metal-containing MMH, a room-temperature viscosity of at least about 15,000 centipoise being required, and 30,000 to 60,000 centipoise being preferred. For the preferred gelling agents given above, 1 to 3 weight percent gelling agent in the mixture is suitable for this purpose. The viscosity can be controlled by varying the amount of gelling agent, higher viscosities being obtained by larger amounts. The amount of gelling agent required to obtain a given viscosity varies somewhat with the physical properties of the metallic particles, smaller amounts being required for particles having a larger surface area.

The term "metallic fuel particles" as used herein is intended to refer to any of the finely divided metals and metal hydrides previously used as fuel in solid propellants. Aluminum, magnesium, boron, beryllium, lead and zirconium and hydrides thereof can be used. The metallic particles must be finely divided in order to remain in suspension and allow pumping of the gel as a liquid, and very fine, generally spherical particles on the order of 6 to 10 microns in diameter are preferred. Platelet-type particles, for example, rectangular shapes 40 by 25 by 0.7 to 0.8 microns in size may also be used. The composition of the metal-containing MMH gel can be varied within wide limits to obtain the performance characteristics desired for a given application. The amount of added metallic particles is selected, depending on the desired trajectory and mission for the particular missile. Up to about 70 weight percent metallic particles can be incorporated in the gel and still allow adequate mixing and pumping as a liquid over a practical range of operating temperatures. For typical applications 20 to 50 weight percent provides maximum overall advantage. The particular metal or hydride is likewise selected, depending on the properties desired. Aluminum and boron are desirable because of their favorable combustion properties and their ready availability in powder form. Beryllium and beryllium hydride provide maximum performance characteristics, but the toxicity of beryllium combustion products limit their usefulness. Lead is preferred for applications requiring maximum density.

The metal-containing MMH gel can be prepared by mixing the metallic particles and the gelling agent with the MMH in a conventional mixer. The gelling agents mentioned above are normally available as finely divided powder which disperses readily in the MMH. The mixing time required for complete dispersion varies

with the particular apparatus and the amount of metallic particles, with longer times being required for larger amounts. Under typical conditions a mixing period of one-half to 2 hours is suitable.

The invention is illustrated by the accompanying drawings wherein:

FIG. 1 is a graph showing calculated specific impulse values for MMH containing varying amounts of aluminum at varying oxidizer-to-fuel ratios, the oxidizer being inhibited red fuming nitric acid.

FIG. 2 is a graph showing calculated specific impulse-density values for the same compositions; any

FIG. 3 is a graph showing the effect of added gelling agent or the viscosity of aluminum-containing MMH.

Referring to FIG. 1, it is seen that specific impulse values are decreased with increasing amounts of aluminum, except at the lowest oxidizer-to-fuel ratios.

FIG. 2 shows that specific impulse-density values are substantially increased with increasing amounts of aluminum. For example, at an oxidizer-to-fuel ratio of 2, the specific impulse-density value increases from less than 370 at 20 weight percent aluminum content to over 400 at 50 weight percent.

FIG. 3 depicts the results obtained by adding varying amounts of hydroxypropyl-substituted cellulose containing 4.6 propoxyl groups per glucose unit (Klucel) to MMH containing 35 weight percent aluminum in the form of spherical particles averaging 6 microns in diameter. Curves A and B show the viscosities in centipoises at varying spindle speeds in standard Brookfield viscosity tests for a 125 milliter portion of the metal-containing MMH with 1.6 and 2.2 weight percent respectively, of gelling agent. In each case the MMH, aluminum and gelling agent were placed in a mixing chamber, and the resulting mixture was agitated for a period of about 1 hour. It is apparent from the curves that a viscosity over 15,000 centipoise, as is required to maintain the particles in suspension, can be obtained by addition of a small amount of gelling agent. The resulting gels were left standing for a period of over 8 months and no settling of particles or other deterioration was observed.

The compositions given in the drawings are merely illustrative and are not to be understood as limiting the scope of the invention, which is limited only as indicated by the appended claims. It is also to be understood that various changes and modifications in appa-

ratus and procedure may be employed by one skilled in the art without departing from the scope of the invention.

What is claimed is:

1. A composition consisting of gelled monomethylhydrazine containing dispersed therein up to 70 weight percent finely divided metallic fuel particles and a cellulose or hydroxyalkyl-substituted cellulose gelling agent.

10 2. The composition of claim 1 wherein said gelling agent is methyl cellulose containing 27.5 to 31.5 weight percent methoxyl groups, hydroxypropyl methyl cellulose containing 28 to 30 weight percent methoxyl groups and 7 to 12 weight percent propoxyl groups, hydroxypropyl methyl cellulose containing 19 to 24 weight percent methoxyl groups and 4 to 12 weight percent propoxyl groups, dihydroxyethyl cellulose or hydroxypropyl cellulose containing about 4.6 propoxyl groups per glucose unit.

3. The composition of claim 2 wherein the amount of said gelling agent is 1 to 3 weight percent.

4. The composition of claim 3 wherein said metallic fuel particles consist of aluminum, magnesium, boron, beryllium, lead, zirconium, aluminum hydride, magnesium hydride, boron hydride, beryllium hydride, lead hydride, or zirconium hydride.

25 5. The composition of claim 4 wherein the amount of said particles is 20 to 50 weight percent.

30 6. The method of preparing a thixotropic monomethylhydrazine gel containing finely divided metallic fuel particles selected from the group consisting of aluminum, magnesium, boron, beryllium, lead, zirconium, aluminum hydride, magnesium hydride, boron hydride, beryllium hydride, lead hydride and zirconium hydride which comprises mixing said particles and said monomethylhydrazine with 1 to 3 weight percent of methyl cellulose containing 27.5 to 31.5 weight percent methoxyl groups, hydroxypropyl methyl cellulose containing 28 to 30 weight percent methoxyl groups and 7 to 12 weight percent propoxyl groups, hydroxypropyl methyl cellulose containing 19 to 24 weight percent methoxyl groups and 4 to 12 weight percent propoxyl groups, dihydroxyethyl cellulose or hydroxypropyl cellulose containing about 4.6 propoxyl groups per glucose unit.

\* \* \* \* \*